

E. C. HISCOCK.  
PROCESS OF VENEERING.  
APPLICATION FILED AUG. 1, 1910.

974,147.

Patented Nov. 1, 1910.

Fig. 1.



Fig. 2.



Witnesses,

S. G. Mann,

S. N. Pond

Inventor,

Emory C. Hiscock

By Offield, Towle, Grans & Offield

Attest.

# UNITED STATES PATENT OFFICE.

EMORY C. HISCOCK, OF CHICAGO, ILLINOIS.

## PROCESS OF VENEERING.

974,147.

Specification of Letters Patent.

Patented Nov. 1, 1910.

Application filed August 1, 1910. Serial No. 575,026.

*To all whom it may concern:*

Be it known that I, EMORY C. HISCOCK, a citizen of the United States, residing at Chicago, in the county of Cook and State of Illinois, have invented a certain new and useful Process of Veneering, of which the following is a specification.

This invention relates to improvements in the art of veneering, and has reference more particularly to a novel method of producing veneered or laminated boards or similar structural parts such as are extensively used by cabinet-makers in the manufacture of articles of high-grade furniture.

15 In the art of veneering as at present extensively practiced, where a very thin veneer, say 1/28 of an inch or less, is cemented either directly on to the body-board, or to an intermediate binder, the glue or other cement employed as an adhesive is, under the enormous pressure to which the structure is subjected, forced into and through the pores of the veneer to such an extent as to render necessary the washing of the outer 20 surface of the veneer preliminary to the finishing operations, and even then the glue shows objectionably in occasional spots and streaks on the outer surface of the veneer even after the final dressing and polishing 25 operations.

One object of my present invention is to eliminate this defect, which I accomplish by filling the veneer from its underside with a solid material rendered plastic by mixture with a volatile vehicle, which material will not injure the tools used in the final dressing of the outer surface and consequently does not require washing of the latter, and which may be colored to correspond substantially with the color to be given the finished surface of the veneer.

Another improvement sought by the invention is to eliminate the tendency of the polished surface of the veneer to split, crack, or craze, which latter defects are mainly attributable to the character of the binder commonly used; and this object I attain through the use of a tough, grainless binder, such as vulcanized fiber. This latter material, which is preferred for the purpose of the invention, is extremely dense, hard and tough, and of uniform texture throughout, and is free from the natural tendency to split or crack, which is characteristic of the ordinary wood binder extensively employed, as well as presenting great tenacity in the

direction of its thickness, so that it is not liable to split in its own plane. This material, vulcanized fiber, also adheres well with the glue or other cement employed as an adhesive; but I have discovered that its quality for uniting perfectly with the glue or other cement is greatly enhanced by preliminarily subjecting it to a bath of acetic acid, as the result of which it forms a joint with the adhesive possessing a degree of cohesion no less than that of the particles of the material of the binder or the veneer itself.

The general object of the invention is to provide an improved process of manufacture which shall result in the production of veneered structures possessing a more perfect finish and surface appearance than any heretofore known, and less subject to deterioration through lapse of time, climatic and atmospheric conditions, and other like causes.

In carrying out my improved method, I cement to the body-board, in the usual way, a binder which consists preferably of a sheet of vulcanized fiber which has preliminarily been treated in a bath of acetic acid, the action of the acid being such as to remove all grease, dirt, and other foreign matter, and put the surface of the binder in a most favorable condition to unite thoroughly with the adhesive employed. Before applying the veneer to said binder, and in lieu of the usual "glue-sizing" which is commonly applied by a brush, I thoroughly rub into the inner surface of the veneer a filler, which must be of such a character that it will adhere perfectly to the glue or other cement used, may be suitably colored in imitation of the color and shade sought for in the finished product, and will also present no obstacle to the subsequent finishing operations, such as the scraping and sanding of the outer surface of the veneer before the outer 100 filler and varnish are applied, and consequently will not require the usual washing operation and subsequent drying, which operations considerably prolong the complete operation. I have found that white lead rendered plastic by mixture with a volatile vehicle, such as benzin, serves this purpose excellently; and this material colored, when necessary, by burnt sienna, Bismarck brown, or any of the known colors, is thoroughly 110 rubbed into the inner surface of the veneer penetrating and filling the pores thereof.

2

The vehicle rapidly evaporates, thus leaving the wood filled with a dry substance, which does not cause any swelling, shrinking, or working of the fibers of the wood, and which 5 at the same time forms with the glue a good adhesive, and, to the extent that it may penetrate to the outer surface of the veneer, presents no obstacle to the subsequent finishing and dressing operations, and does not render 10 it necessary to wash the outer surface of the veneer before the finishing and dressing operations. The veneer thus filled is applied and adhered to the binder under pressure in the usual manner. The veneered structure 15 is then allowed to dry out under ordinary atmospheric temperatures; it is then, without washing, put through the usual cabinet operations of trimming, scraping, and sanding; and finally the exposed surface of the 20 veneer is subjected to some or all of the usual finishing operations consisting of filling, staining, varnishing, rubbing, polishing, and oiling off. The result is a veneered structure possessing a finished surface of 25 great perfection and durability in respect to its appearance, and one which will remain permanently free from the defects of cracking, crazing, warping, and other indications 30 of deterioration commonly seen in ordinary veneers. This superior result is due in part to the character of the binder employed; in part to the preliminary treatment of the binder in an acid bath; in part to the exclusion 35 of the glue or other cement from the pores of the veneer by the solid filler that is preliminarily applied to the inner side of the veneer before the same is adhered to the binder; and in part to the elimination of the washing operation.

40 To render the disclosure of my invention fuller and more complete I have illustrated in the accompanying drawing a structure made in accordance with the present invention, Figure 1 showing the same in top plan view with the several laminations thereof 45 broken off at different points, and Fig. 2 showing a vertical longitudinal section of Fig. 1.

In the said drawing 1 represents the body 50 board, 2 the layer of glue or other cement applied to the surface thereof, 3 the binder consisting, as stated, of tough, dense grain-

less material such as vulcanized fiber, 4 the 55 layer of glue or other cement applied to the upper surface of said binder, 5 the veneer filled from its underside with a plastic filler such as white lead, thoroughly rubbed into the same, said filler being indicated at 6, 60 and 7 the outer varnished and polished surface.

I claim:—

1. The process of manufacturing veneered structures which consists in cementing a 65 binder to the body-board, rubbing into the veneer from its inner side a plastic filler, cementing said veneer to the binder and finishing the outer side of the veneer.

2. The process of manufacturing veneered 70 structures which consists in cementing a binder to the body-board, rubbing into the veneer from its inner side a plastic filler, cementing said veneer to the binder, and then, without washing, subjecting the outer 75 surface of the veneer to the usual finishing operations.

3. The process of manufacturing veneered structures which consists in subjecting a 80 grainless fibrous binder to an acid bath, cementing said binder to the body-board, rubbing into the veneer from its inner side a solid filling material rendered plastic by mixture with a volatile vehicle, cementing 85 said veneer to the binder, and finishing the outer side of the veneer.

4. The herein described process of manufacturing veneered structures which consists in subjecting a binder of vulcanized fiber to an acid bath, cementing said binder to the 90 body-board, rubbing into the veneer from its inner side a white lead filler rendered plastic by mixture with a volatile vehicle, cementing said veneer to the binder, allowing the structure to dry at atmospheric temperatures, and 95 then, without washing, subjecting the outer surface of the veneer to the usual finishing operations.

In testimony that I claim the foregoing as my invention, I have hereunto subscribed 100 my name in the presence of two witnesses.

EMORY C. HISCOCK.

Witnesses:

SAMUEL N. POND,  
DAISY C. THORSEN.